

## UNITED STATES PATENT OFFICE

2,666,738

## BRIGHT SILVER PLATING

Otto Kardos, Keyport, N. J., assignor to Hanson-Van Winkle-Munning Company, Matawan, N. J., a corporation of New Jersey

No Drawing. Application September 15, 1950,  
Serial No. 185,171

10 Claims. (Cl. 204—46)

1

This invention relates to silver plating and more particularly to the electrodeposition of bright silver deposits from silver cyanide plating baths.

I have discovered that reaction products of ketones, especially of acetone, methyl ethyl ketone and acetonylacetone (2,5-hexanedione) with carbon disulfide and alkali hydroxide, when properly purified, are excellent brighteners for cyanide silver solutions.

I have further discovered that these ketone-carbon disulfide reaction products cooperate very strongly with small amounts of Turkey red oil (sulfonated castor oil), if the concentration of the latter is maintained within rather narrow limits.

Various sulfur-containing compounds such as: carbon disulfide, ammonium thiosulfate, potassium ethyl xanthogenate, thiourea, alkali dithiocarbamates, mercaptobenzothiazole, mercaptothiazole and mercaptothiazoline have been proposed and used as silver brighteners. Also the simultaneous use of Turkey red oil with potassium xanthogenate and of Turkey red oil with carbon disulfide as addition agents has been proposed.

A thorough examination of these addition agents, as well as many other sulfur-containing compounds such as: beta-Mercaptoethanol, 2-mercaptoethyl pyridine, ethylene thiourea, di-thiobiuret, rhodanine (2-thiono-4-keto-thiazolidine), 2,4-diketothiazolidine, thioammeline, di-thioammeline, 2,4-diamino-6-thio-1,3,5-thiadiazine and various alkali soluble ammonium thiocyanate-formaldehyde resins, showed that the addition of the above agents, alone or with Turkey red oil, did not give as brilliant a silver deposit as the deposit from a silver plating bath containing the ketone-carbon disulfide reaction products. The ketone-carbon disulfide reaction products in a silver plating bath also permitted the use of a wider current density range and the bath was more stable.

The reaction of ketones of the general type  $\text{RCH}_2\text{COCH}_2\text{R}$  and carbon disulfide in the presence of powdered potassium hydroxide has been described by Apitzsch, Ber. 37, 1,599 (1904); 38, 2,888 (1905) and 41,4028 (1908).

I have extended this reaction to the gamma diketone acetonylacetone (2,5-hexanedione), and have found that the reaction proceeds also in presence of a 50% solution of aqueous sodium hydroxide; slowly for acetone and methyl ethyl ketone, rapidly for acetonylacetone. I have also found that these reaction products are able to react with formaldehyde.

2

For the application as silver brighteners, it is very important that the sodium sulfide (or hydrosulfide) formed by this reaction is completely eliminated from the ketone-carbon disulfide reaction products before their addition to the silver plating bath. This is done by acidulating the end product of this reaction with mineral acid, whereby, the ketone-carbon disulfide reaction product precipitates and hydrogen sulfide is formed. The precipitate is then thoroughly washed with water, redissolved in dilute aqueous sodium hydroxide and reprecipitated with acid. This purification of the reaction product by dissolution in dilute aqueous sodium hydroxide and precipitation with mineral acid can be repeated several times. The final product can be dried in vacuo and powdered. Weaker acids, such as acetic acid, do not precipitate these reaction products. However, after boiling away the hydrogen sulfide, such solutions can also be used as silver brighteners.

A preferred formula for an aqueous silver bath is:

|                     | oz./gal. |
|---------------------|----------|
| Silver cyanide      | 8.0      |
| Potassium cyanide   | 18.0     |
| Potassium carbonate | 6.0      |
| Potassium hydroxide | 0.4      |

But obviously this is but one example of many possible bath formulas. When, to such a bath, 0.02 to 0.04 oz./gal. of a methyl ethyl ketone-carbon disulfide reaction product, or of an acetonylacetone-carbon disulfide reaction product, were added together with 10 ml./l. of Turkey red oil (50%), excellent silver electrodeposits were obtained in the Hull cell over a wide current density range. But after about one day's standing or use of the bath, the degree of brightness of the electrodeposits is considerably reduced and the current density range of brightness considerably narrowed and it is not possible to restore the excellent initial bath performance by addition of ketone-carbon disulfide reaction product, Turkey red oil or other bath components. It has been found that if only 0.8 ml./l. of Turkey red oil (50%) is used, together with 0.02 to 0.04 oz./gal. of ketone-carbon disulfide reaction product, there occurs, on standing of the bath, first an improvement of the bath performance, followed by a slow decrease of the brilliancy of the silver deposit; but the brightness range is not narrowed. In this case, that is when only 0.8 ml./l. of Turkey red oil (50%) have been added, the initial excellent bath performance can be easily restored by the addition of small amounts

of the ketone-carbon disulfide reaction product, approximately 0.01 oz./gal. per week of standing. Addition of only 0.4 ml./l. of Turkey red oil (50%) to a silver bath containing 0.02 to 0.04 oz./gal. of ketone-carbon disulfide reaction product, initially produces matte and streaky silver deposits. An improvement is noticed if the bath has been standing for several hours. The presence of 1.6 ml./l. of Turkey red oil (50%) will, upon standing, gradually narrow the brightening range of the electrodeposits. The limits for the concentration of Turkey red oil, for continuous satisfactory bath performance, are between 0.4 ml./l. and 1.6 ml./l. or preferably 0.6 ml./l. to 1.2 ml./l. of Turkey red oil (50%).

It should be recorded that some of the methyl ethyl ketone-carbon disulfide reaction products produced excellent silver electrodeposits over a wide current density range, even in absence of Turkey red oil, and that all ketone-carbon disulfide reaction products produced, in absence of Turkey red oil, at least semi-bright silver electrodeposits in an unagitated bath; their brightness was strongly increased by agitation. However, in order to obtain maximum brightness, the addition of 0.6 to 1.2 ml./l. of Turkey red oil (50%) to the silver plating bath is generally desirable.

#### Example 1

22.8 g. (0.2 mol) acetonylacetone  
61 g. (0.8 mol) carbon disulfide  
96 g. (1.2 mols) aqueous sodium hydroxide solution (50%)

were put into a closed bottle or flask supplied with reflux condenser.

On occasional shaking, the two-phase reaction mixture darkened, a moderate heat evolution occurred and after about 45 minutes the mixture was homogeneous, dark red-brown and fairly warm. The mixture was then cooled to room temperature and diluted with 400 ml. of water. 1.2 mols of hydrochloric acid (1:1 by volume) were then slowly added under stirring. An almost black resinous mass was precipitated and much hydrogen sulfide escaped. The precipitate was powdered, washed with water and redissolved with 0.8 mol of aqueous sodium hydroxide. This solution was then diluted to approximately 500 ml., and 0.8 mol of hydrochloric acid (1:1 by volume) were added under stirring. The dark brown precipitate was filtered off, washed with water and air or vacuum dried. 0.02 oz./gal. of this reaction product, when added to the silver bath as described above, gave a semi-bright silver deposit in the Hull cell up to about 20 amps./sq. ft. On addition of 0.8 ml./l. (0.1 fl. oz./gal.) of Turkey red oil (50%), a brilliant silver deposit was obtained in the Hull cell up to 20 amps./sq. ft. On agitation in a beaker, brilliant silver deposits were obtained up to 45 amps./sq. ft.

Addition of only 0.4 ml./l. of Turkey red oil (50%) gave at first a matte irregular silver electrodeposit, and only after several hours' standing could fair deposits be obtained. With 1.6 ml./l. of Turkey red oil, the bath showed some deterioration of performance on standing, and could not be restored to its initial good performance.

In a more dilute bath prepared from

oz./gal.  
Silver cyanide ..... 6.0  
Potassium cyanide ..... 14.0  
Potassium carbonate ..... 4.5  
Potassium hydroxide ..... 0.4

oz./gal.  
Acetonylacetone-carbon disulfide reaction product ..... 0.02  
Turkey red oil (50%) 0.1 fl. oz./gal.

5 bright silver deposits up to 30 amp./sq. ft. could be obtained only with strong mechanical agitation of the bath.

For the preparation of small amounts of acetonyl-acetone-carbon disulfide-alkali hydroxide reaction product, temperature control is not required as the reaction is moderately fast and exothermic and the upper temperature range is limited by the boiling point of carbon disulfide. For the preparation of larger amounts of reaction product, strong cooling of the reaction mixture is required after an initial induction period of about 45 to 60 minutes, so that the reaction does not become too violent. For highest yields of solid reaction product, final maintenance of the reaction mixture at 50° C. for several hours, before precipitation with acid, is useful.

#### Example 2

25 0.2 mol acetonylacetone  
0.8 mol carbon disulfide  
1.2 mols aqueous sodium hydroxide solution (50%)

30 reacted as in Example 1.

Then, after dilution to 600 ml., instead of hydrochloric acid, slightly over 1.2 mols of acetic acid were added. The solution was boiled down to 400 ml., neutralized with potassium hydroxide solution, diluted to 600 ml. and filtered. 8 ml. of this dark red brightener solution, when added to 1 liter silver bath, produced bright silver electrodeposits up to about 20 amps./sq. ft. in the Hull cell, the brightness of which was further increased by addition of 0.8 ml./l. Turkey red oil (50%).

On standing, the brightener stock solution deteriorates slowly, apparently by formation of sodium sulfide but can be restored to its initial performance by acidulation with acetic acid, boiling and neutralization.

#### Example 3

50 0.2 mol acetonylacetone  
0.8 mol carbon disulfide  
1.2 mols aqueous sodium hydroxide solution (50%)

reacted as in Example 1.

After the mixture had become homogeneous, it 55 was cooled to room temperature and 0.1 mol (7.5 ml.) of aqueous formaldehyde (37%) was added. An exothermic reaction occurred, and after about 15 minutes the reaction mass was cooled, diluted and precipitated as in Example 1. A black resinous lump precipitated, was washed with water and hardened on standing overnight. It was powdered, dissolved in aqueous sodium hydroxide, precipitated with dilute hydrochloric acid (1:1 by volume) in an amount at least equivalent to the sodium hydroxide used, filtered, washed, redissolved in aqueous sodium hydroxide and reprecipitated with hydrochloric acid. After air drying, 19.5 grams of a light brown powder were obtained. The results obtained with this 60 addition agent in a silver bath were the same as those obtained with the addition agent described in Example 1. Similarly effective addition agents were obtained by using 1.6 instead of 1.2 mols of sodium hydroxide, or by using 0.2 mol of formaldehyde instead of 0.1 mol.

70 75

*Example 4*

14.4 g. (0.2 mol) methyl ethyl ketone  
 30.5 g. (0.4 mol) carbon disulfide  
 48.0 g. (0.6 mol) aqueous sodium hydroxide solution (50%)

The above was shaken occasionally in a closed bottle for about two weeks, after which time the mixture became homogeneous. Then 7.5 ml. (0.1 mol) of formaldehyde (37%) were added and, after standing for about 15 minutes, an addition of 300 ml. of water and finally 0.6 mol of glacial acetic acid were made. The solution was heated to drive out all hydrogen sulfide; and after addition of 0.6 mol of sodium hydroxide it was diluted to 400 ml. 4 ml. of this brightener solution, when added to 1 liter of silver bath, produced bright silver electrodeposits over a wide current density range. Their brightness was further increased by addition of 0.8 ml./l. of Turkey red oil (50%).

*Example 5*

25 g. (0.35 mol) methyl ethyl ketone  
 100 g. (1.31 mol) carbon disulfide  
 75 g. (1.33 mol) potassium hydroxide (powdered)  
 1 ml. water

The above mixture was heated under reflux for 4 hours on a water bath. The liquid was poured off from the dark red solid mass and the latter dissolved in 200 ml. of water. Then 230 ml. of hydrochloric acid (1:1 by volume) were slowly added under stirring. A black resin pitch precipitated, which was dissolved in 20 ml. of sodium hydroxide solution (20%), reacted with 15 ml. of formaldehyde (37%), precipitated with dilute hydrochloric acid and, after filtering, redissolved in sodium hydroxide and precipitated again with hydrochloric acid. A brown powder resulted which, after washing with water and air drying, was used as an addition agent to the standard silver bath. 0.04 oz./gal. of this product produced brilliant silver deposits in the Hull cell and in a beaker at up to 30 amps./sq. ft. with agitation. Similar brighteners were prepared without the use of formaldehyde. In general, the presence of formaldehyde will facilitate the formation of the final products in powder form and increase the yield of these reactions.

*Example 6*

10.5 g. (0.145 mol) methyl ethyl ketone  
 19 g. (0.25 mol) carbon disulfide  
 22 g. (0.39 mol) potassium hydroxide (powder), and  
 7.5 to 25 g. dimethoxytetraglycol

The above were reacted in a flask under reflux.

The presence of dimethoxytetraglycol accelerated the reaction considerably. After about 15 minutes, the brown reaction product was dissolved in 200 ml. of water. This solution was then acidulated with 25 ml. of glacial acetic acid, evaporated to two-thirds of its volume, neutralized with an aqueous solution of potassium hydroxide, diluted to 400 ml. and filtered. A volume of 24 to 40 ml. of this solution, when added to the standard silver bath, caused the formation of bright silver deposits over a wide current density range. The appearance of the silver deposit was further improved on addition of 0.8 ml./l. of Turkey red oil (50%).

Some batches of brighteners prepared similar to Examples 4, 5 and 6 gave full bright silver electrodeposits even in absence of Turkey red oil.

Other batches gave brilliant silver deposits only in presence of small amounts of Turkey red oil. Also, the presence of Turkey red oil increases the tarnish resistance of the silver electrodeposits.

5 Here again, with 10 ml./l. of Turkey red oil (50%), the deposits were excellent in the beginning, but the current density range over which brightness could be obtained narrowed considerably after a few hours' standing of the bath, and the initial wide brightness range could not be restored by any additions. With only 0.8 ml./l. of Turkey red oil (50%), the bath performance remained fairly stable and could be completely restored by small periodic additions of ketone-carbon disulfide brightener.

Similar addition agents were obtained from acetone instead of methyl ethyl ketone.

The carbon disulfide reaction products of diethyl ketone, methylamyl ketone, mesityl oxide and of sodium levulinate ( $\text{CH}_3\text{COCH}_2\text{CH}_2\text{COONa}$ ) gave somewhat less satisfactory brighteners.

Acetylacetone and acetol reacted very violently with sodium hydroxide (50%) and carbon disulfide, and were thus not suitable as starting materials.

25 As far as the ease of obtaining these addition agents in solid form of reproducible brightening efficiency and in reasonably good yield is concerned, I prefer the acetylacetone-carbon disulfide reaction products as described in Examples 1 and 3.

I claim:

1. A process for producing bright silver electrodeposits, which comprises electrodepositing silver from an aqueous cyanide silver plating bath containing 0.02 to 0.04 oz./gal. (0.15 to 0.30 g./liter) of the solid, water- and acid insoluble but alkali soluble reaction product of a ketone of the formula  $\text{RCH}_2\text{COCH}_3$ , where R comprises a substituent selected from the group consisting of hydrogen, alkyl, acetyl (CH<sub>3</sub>COCH<sub>2</sub>—) and alkali metal carboxymethyl (—CH<sub>2</sub>COONa, —CH<sub>2</sub>COOK), with carbon disulfide and alkali hydroxide, this reaction product having been precipitated by addition of a strong mineral acid and freed from alkali sulfide and hydrogen sulfide.

2. A process for producing bright silver electrodeposits, which comprises electrodepositing silver from an aqueous cyanide silver plating bath containing 0.4 to 1.6 ml./l. of an aqueous solution of Turkey red oil, 50%, and 0.02 to 0.04 oz./gal. (0.15 to 0.30 g./liter) of the solid, water- and acid insoluble but alkali soluble reaction product of a ketone of the formula  $\text{RCH}_2\text{COCH}_3$ , where R comprises a substituent selected from the group consisting of hydrogen, alkyl, acetyl

(CH<sub>3</sub>COCH<sub>2</sub>—)

and alkali metal carboxymethyl (—CH<sub>2</sub>COONa, —CH<sub>2</sub>COOK), with carbon disulfide and alkali hydroxide, this reaction product having been precipitated by addition of a strong mineral acid and freed from alkali sulfide and hydrogen sulfide.

3. A process for producing bright silver electrodeposits, which comprises electrodepositing silver from an aqueous cyanide silver plating bath containing 0.02 to 0.04 oz./gal. (0.15 to 0.30 g./liter) of the solid, water- and acid insoluble but alkali soluble reaction product of a ketone of the formula  $\text{RCH}_2\text{COCH}_3$ , where R comprises a substituent selected from the group consisting of hydrogen, alkyl, acetyl (CH<sub>3</sub>COCH<sub>2</sub>—) and alkali metal carboxymethyl

(—CH<sub>2</sub>COONa, —CH<sub>2</sub>COOK)

with substantially two mols carbon disulfide per mol carbonyl group and at least one and a half mols alkali hydroxide per mol carbon disulfide, this reaction product having been precipitated by addition of a strong mineral acid and freed from alkali sulfide and hydrogen sulfide.

4. A process for producing bright silver electrodeposits, which comprises electrodepositing silver from an aqueous cyanide silver plating bath containing 0.4 to 1.6 ml./l. of an aqueous solution of Turkey red oil, 50%, and 0.02 to 0.04 oz./gal. (0.15 to 0.30 g./liter) of the solid, water- and acid insoluble but alkali soluble reaction product of a ketone of the formula  $RCH_2COCH_2$ , where R comprises a substituent selected from the group consisting of hydrogen, alkyl, acetonyl



and alkali metal carboxymethyl



with substantially two mols carbon disulfide per mol carbonyl group and at least one and a half mols alkali hydroxide per mol carbon disulfide, this reaction product having been precipitated by addition of a strong mineral acid and freed from alkali sulfide and hydrogen sulfide.

5. A process for producing bright silver electrodeposits, which comprises electrodepositing silver from an aqueous cyanide silver plating bath containing 0.02 to 0.04 oz./gal. (0.15 to 0.30 g./liter) of the solid, water- and acid insoluble but alkali soluble reaction product of a ketone, selected from a group consisting of acetonyl acetone, methyl ethyl ketone and acetone, with carbon disulfide and alkali hydroxide, this reaction product having been precipitated by addition of a strong mineral acid and freed from alkali sulfide and hydrogen sulfide.

6. A process for producing bright silver electrodeposits, which comprises electrodepositing silver from an aqueous cyanide silver plating bath containing 0.4 to 1.6 ml./l. of an aqueous solution of Turkey red oil, 50%, and 0.02 to 0.04 oz./gal. (0.15 to 0.30 g./liter) of the solid, water- and acid insoluble but alkali soluble reaction product of a ketone, selected from a group consisting of acetonylacetone, methyl ethyl ketone and acetone, with carbon disulfide and alkali hydroxide, this reaction product having been precipitated by addition of a strong mineral acid and freed from alkali sulfide and hydrogen sulfide.

7. A process for producing bright silver electrodeposits, which comprises electrodepositing silver from an aqueous cyanide silver plating bath containing 0.02 to 0.04 oz. gal. (0.15 to 0.30 g./liter) of the solid, water- and acid insoluble but alkali soluble reaction product of a ketone, selected from a group consisting of acetonylacetone, methyl ethyl ketone and acetone, with substantially two mols carbon disulfide per mol carbonyl group and at least one and a half mols alkali hydroxide per mol carbon disulfide, this reaction product having been precipitated by addition of a strong mineral acid and freed from alkali sulfide and hydrogen sulfide.

8. A process for producing bright silver electrodeposits, which comprises electrodepositing silver from an aqueous cyanide silver plating bath containing 0.4 to 1.6 ml./l. of an aqueous solution of Turkey red oil, 50%, and 0.02 to 0.04 oz./gal. (0.15 to 0.30 g./liter) of the solid, water- and acid insoluble but alkali soluble reaction product of a ketone, selected from a group consisting of acetonylacetone, methyl ethyl ketone and acetone, with substantially two mols carbon disulfide per mol carbonyl group and at least one and a half mols alkali hydroxide per mol carbon disulfide, this reaction product having been precipitated by addition of a strong mineral acid and freed from alkali sulfide and hydrogen sulfide.

9. A process for producing bright silver electrodeposits, which comprises electrodepositing silver from an aqueous cyanide silver plating bath containing 0.02 to 0.04 oz./gal. (0.15 to 0.30 g./liter) of the solid, water- and acid insoluble but alkali soluble reaction product of a ketone, selected from a group consisting of acetonylacetone, methyl ethyl ketone and acetone with substantially two mols carbon disulfide per mol carbonyl group and at least one and a half mols alkali hydroxide, in the form of a concentrated aqueous solution, per mol carbon disulfide, this reaction having been allowed to proceed between 30 and 50° C. at least until the initially heterogeneous reaction mixture became homogeneous and this reaction product having been precipitated by addition of a strong mineral acid and freed from alkali sulfide and hydrogen sulfide.

10. A process for producing bright silver electrodeposits, which comprises electrodepositing silver from an aqueous cyanide silver plating bath containing 0.4 to 1.6 ml./l. of an aqueous solution of Turkey red oil, 50%, and 0.02 to 0.04 oz./gal. (0.15 to 0.30 g./liter) of the solid, water- and acid insoluble but alkali soluble reaction product of a ketone, selected from a group consisting of acetonylacetone, methyl ethyl ketone and acetone with substantially two mols carbon disulfide per mol carbonyl group and at least one and a half mols alkali hydroxide, in the form of a concentrated aqueous solution, per mol carbon disulfide, this reaction having been allowed to proceed between 30 and 50° C. at least until the initially heterogeneous reaction mixture became homogeneous and this reaction product having been precipitated by addition of a strong mineral acid and freed from alkali sulfide and hydrogen sulfide.

OTTO KARDOS.

References Cited in the file of this patent

UNITED STATES PATENTS

| Number    | Name                | Date          |
|-----------|---------------------|---------------|
| 2,110,792 | Egberg et al. ----- | Mar. 8, 1938  |
| 2,113,517 | Powell et al. ----- | Apr. 5, 1938  |
| 2,176,668 | Egberg et al. ----- | Oct. 17, 1939 |

OTHER REFERENCES

65 Ser. No. 351,241, Weiner (A. P. C.), published May 18, 1943.